

Dec. 14, 1943.

N. H. BJERG ET AL

2,337,012

STENCIL SHEETS AND METHOD OF MAKING SAME

Filed March 11, 1941

Fig. 1.



Fig. 2.



INVENTORS  
Niels Holger Bjerg and Albert B. Ulrich Jr.  
BY  
Byerly, Watson and Simonds  
ATTORNEYS

## UNITED STATES PATENT OFFICE

2,337,012

STENCIL SHEET AND METHOD OF  
MAKING SAME

Niels Holger Bjerg, Chicago, and Albert B. Dick,  
Jr., Lake Forest, Ill., assignors to A. B. Dick  
Company, Chicago, Ill., a corporation of Il-  
linois

Application March 11, 1941, Serial No. 382,690

16 Claims. (Cl. 101—128.2)

This invention relates to stencil sheets and method of making same, and aims to provide a stencil sheet perfectly adapted both to stencilization with a stylus and to stencilization in a typewriter.

A stencil sheet for making a stencil for use in a duplicating machine consists of an open, porous, fibrous base having a displaceable coating filling the interstices of the base. A common base is yoshino paper. The usual coating consists essentially of a binding agent and softening agents. The nature and more particularly the proportion of the two agents determine the physical characteristics of the coating, which must be such as to make it displaceable by pressure applied to the sheet.

In preparing duplicating stencils from stencil sheets, it is customary to use a stylus for drawing and signatures and the type of a typewriter for text. The pressure which a stencil receives from a stylus is very different from the blow which it receives in a typewriter. It has long been recognized that in order to be well adapted for stencilization with a stylus, a stencil sheet should have a coating which is soft and fluent, so that it may be readily displaced by drawing a stylus across the sheet. It has also been recognized that the most satisfactory stencil sheets for stencilization in a typewriter are those which have a relatively hard coating, which, while readily displaceable by a blow of the type, is not soft and fluent enough to fill the type of the typewriter and thus necessitate frequent cleaning of the type. It has proved impossible heretofore to provide a stencil sheet with a coating which is both soft and fluid enough to stencilize well with a stylus and hard enough to avoid any filling of the typewriter type struck against it.

By our invention we have succeeded in producing a stencil sheet combining the antagonistic qualities desired for stylus stencilization and type stencilization. We have accomplished this by providing a stencil sheet with a coating which, while unitary, is non-uniform and has different physical characteristics at the two sides of the sheet. At one side of the sheet the coating has the soft and fluid characteristic required for stencilization with a stylus. At the other side, the coating is relatively hard and non-fluent, so that when the sheet is struck by type on this

side, it does not fill the type. The non-uniform coating is formed by the amalgamation of two compatible layers—a relatively hard layer located mostly within the confines of the base, and a relatively fluent layer located mostly at one side of the base.

Our method of making such a stencil sheet consists in first impregnating a porous base with a thin, fast-drying solution producing a 10 relatively hard layer within the base. After this layer has nearly, but not completely, dried, the impregnated base is coated with a thicker, slow-drying solution which is compatible with the first solution. This leaves on one side of the base 15 a relatively fluent layer. The two layers, being compatible, amalgamate by interpenetration, producing a unitary rather than a laminated coating. But, notwithstanding the amalgamation which eliminates any definite line of demarcation, 20 the different physical characteristics of the two layers are retained at the two sides of the amalgamated coating.

In order that the two coating solutions may be compatible and may produce layers which amalgamate, it is essential that the binding agents in both solutions be soluble in the solvent used in the second solution. Most desirably the two solutions contain the same solvent and the same binding agent and compatible or identical softening agents.

In describing our invention in detail, we shall refer to the accompanying drawing in which Figs. 1 and 2 are diagrammatic cross-sections of a stencil sheet showing the effect of the two steps 35 of our method.

In the drawing, 10 represents the base sheet consisting of fibers 11, projecting beyond the general surface of the sheet in the form of a fuzz 12 which is easily discernible to the eye and to the touch.

The first step in making the stencil sheet consists in impregnating the base 10 with a first coating solution containing a binding agent, softening agents and a volatile solvent in which the 45 binding agent is dissolved. The proportion and nature of the softening agents is so adjusted that the solution will deposit a film or layer harder than an ordinary stencil coating, but soft enough to be displaced by a blow of the type in a typewriter. A large proportion of volatile solvent is

used so as to make the solution quick-drying. The impregnation of the base 10 with the solution may be effected in any well known manner as by a coating roller or wheel or by floating the base on the surface of a bath and then pulling it over a rod. The thin, highly volatile coating solution quickly strikes through or almost through the base from the side to which it is applied. This is the under side of the sections shown in the drawing. This solution with which the base has been impregnated dries so rapidly that the ends of the fibers forming the fuzz 12 still project from the upper surface of the sheet 10, so that after drying, this side of the sheet still has a slightly rough feel. Thus, as seen in Fig. 1, the effect of the first coating operation is to leave in the base a layer 20 of coating material, most of which is within the confines of the base. This layer extends from slightly outside the under surface of the sheet to which the solution was applied, to slightly inside the extreme upper surface of the sheet.

The softening agent of the solution is partially absorbed into the fibers 11 of the base 10, so that the ratio of binding agent to softening agents in the material deposited between the fibers is somewhat higher than it was in the solution. This effect as well as the composition of the solution makes the layer 20 harder and less fluent than an ordinary stencil coating.

Being almost wholly within the confines of the porous base sheet 10, the layer 20 to some extent strengthens the fibrous sheet, acting in this respect as a sizing.

After the layer left in the base by the first coating operation is nearly dry but while it still contains sufficient solvent to be very soft, the second coating solution is applied to the under side of the base. This solution also contains a binding agent, softening agents and a solvent in which the binding agent is dissolved. The ingredients are adjusted so as to deposit a soft and fluent material, and only a moderate amount of solvent is used so that the second solution is thicker than the first solution and dries more slowly. The second solution leaves on the under surface of the base a layer 30 which is shown in Fig. 2.

During the application of the second solution, the solvent of the second solution penetrates into the layer deposited by the first solution and an intermingling of the two layers continues until all the solvent has evaporated. The two layers therefore coalesce so that there is no line of demarcation between them. However, none of the second layer passes completely through the first layer to the upper side of the base. As a result, the amalgamated coating retains the physical characteristics of the first layer at the upper side of the sheet and those of the second layer at the lower side. A further result is that no part of the complete amalgamated coating projects beyond the confines of the projecting fibers at the upper side of the sheet.

The fluent character of the coating at its lower side and indeed throughout its main body, makes the stencil sheet ideally adapted to stencilization by a stylus. At the same time the hardness of the coating at the upper side of the sheet effectively prevents filling of the type when the type strikes this side of the sheet in stencilizing the sheet in a typewriter. This desirable result is also insured by the fact that no part of the coating projects beyond the fibers at the upper side of the sheet. The new stencil

sheet therefore meets the most rigid requirements both of a sheet to be stencilized by a stylus and of a sheet to be stencilized in a typewriter.

5 The coating solutions used in carrying out our method may consist of the ingredients commonly used in stencil sheet coating. The compounding of such solutions so as to deposit films or layers of different degrees of softness is well understood 10 in the stencil sheet art. To illustrate the scope of our invention, we give a few illustrative formulae of coating solutions which deposit films or layers of the character required by our method.

We find it most desirable to use nitrocellulose 15 as the binding agent and a mixture of ether and alcohol as the solvent in both the first and second solutions. Satisfactory compositions for the two solutions are as follows:

#### EXAMPLE I

##### First solution

|                | Parts by weight |
|----------------|-----------------|
| Nitrocellulose | 300             |
| Alcohol        | 8,300           |
| Ether          | 10,900          |
| Castor oil     | 1,125           |
| Stearic acid   | 250             |
| Benzyl alcohol | 100             |
| Triacetin      | 150             |

30 This is a thin, highly volatile solution which dries rapidly and produces a displaceable but relatively hard coating.

##### Second solution

|                 | Parts by weight |
|-----------------|-----------------|
| Nitrocellulose  | 120             |
| Alcohol         | 920             |
| Ether           | 1,960           |
| Amyl stearate   | 500             |
| Color (pigment) | 100             |

35 This is a normal solution for producing a relatively thick coating of a soft and fluent character.

When it is desired to apply our method to 45 making a stencil sheet whose coating has a protein binder, the following compositions will be found to be satisfactory:

#### EXAMPLE II

##### First solution

|             | Parts by weight |
|-------------|-----------------|
| Gelatin     | 100             |
| Glycerol    | 20              |
| Mineral oil | 500             |
| Water       | 5,000           |

##### Second solution

|                 | Parts by weight |
|-----------------|-----------------|
| Gelatin         | 200             |
| Glycerol        | 50              |
| Sulphonated oil | 150             |
| Mineral oil     | 800             |
| Wax             | 300             |
| Pigment         | 300             |
| Water           | 3,400           |

60 In this case, each bath contains the binding agent, gelatin, dissolved in the solvent, water.

While it is desirable to use the same binder in both solutions so as to insure a thorough amalgamation of the two layers, this is not absolutely essential in the practice of the invention. Different binding agents may be used in the two solutions provided that the solvent of the second solution is capable of dissolving both the

binding agents. This is the case in the following examples:

EXAMPLE III

*First solution*

|                | Parts by weight |
|----------------|-----------------|
| Nitrocellulose | 300             |
| Alcohol        | 8,300           |
| Ether          | 10,900          |
| Castor oil     | 1,125           |
| Stearic acid   | 250             |
| Benzyl alcohol | 100             |
| Triacetin      | 150             |

*Second solution*

|                     | Parts by weight |
|---------------------|-----------------|
| Gelatin             | 200             |
| Glycerol            | 50              |
| Sulphonated oil     | 150             |
| Mineral oil         | 800             |
| Wax                 | 300             |
| Pigment             | 300             |
| Glacial acetic acid | 3,400           |

EXAMPLE IV

*First solution*

|             | Parts by weight |
|-------------|-----------------|
| Gelatin     | 100             |
| Glycerol    | 20              |
| Mineral oil | 500             |
| Water       | 5,000           |

*Second solution*

|                     | Parts by weight |
|---------------------|-----------------|
| Nitrocellulose      | 120             |
| Glacial acetic acid | 2,880           |
| Amyl stearate       | 500             |
| Color (pigment)     | 100             |

What we claim is:

1. A stencil sheet adapted to be made into a stencil by a typewriter or by a stylus and comprising a porous base having a unitary but non-uniform displaceable coating which is relatively hard at one side of the sheet and relatively soft and fluent at the other side.

2. A stencil sheet comprising a porous base having a unitary displaceable coating consisting of a binding agent and softening agents, the ratio of binding agent to softening agents being greater at one side of the sheet than at the other.

3. A stencil sheet comprising a porous base having a unitary displaceable coating consisting of a cellulose compound and softening agents, the ratio of cellulose compound to softening agents being greater at one side of the sheet than at the other.

4. A stencil sheet comprising a porous base having a unitary displaceable coating consisting of a protein and softening agents, the ratio of protein to softening agents being greater at one side of the sheet than at the other.

5. A stencil sheet comprising a porous base having a unitary but non-uniform displaceable coating consisting of a cellulose compound, a protein and softening agents, which is relatively hard at one side of the sheet and relatively soft and fluent at the other side.

6. A stencil sheet comprising a porous paper base and a displaceable coating of nitrocellulose and softening agents impregnating said base and projecting beyond the fibers of the base at one side of the base only.

7. A stencil sheet comprising a porous fibrous base having a unitary displaceable coating consisting of a relatively hard sizing layer and a relatively soft external layer, said layers being compatible and merging into one another.

8. A stencil sheet comprising a porous fibrous base having a unitary but non-uniform displaceable coating consisting of a relatively hard sizing layer of binding agent and softening agents and a relatively soft external layer of the same binding agent and compatible softening agents, said layers merging into one another.

9. The method of making a stencil sheet which comprises successively applying to an open base of porous fibres a quick-drying solution containing binder and softener and a compatible slow-drying solution containing binder and softener.

10. The method of making a stencil sheet which comprises successively applying to an open base of porous fibres two solutions each containing volatile solvent, binder and softener, the solution first applied containing a relatively large proportion of volatile solvent and the second solution containing a relatively small proportion of the same volatile solvent.

11. The method of making a stencil sheet which comprises successively applying to a porous base a coating solution so compounded as to deposit a relatively hard type-impressible film and a compatible solution so compounded as to deposit a relatively soft and fluent type-impressible film.

12. The method of making a stencil sheet which comprises impregnating an open base of porous fibres with a relatively thin solution of a binding agent containing softening agents, and thereafter coating one side of the impregnated base with a relatively thick solution of a binder containing softening agents, the solvent of the second solution being capable of dissolving the binder of the first solution.

13. The method of making a stencil sheet which comprises successively applying to an open base of porous fibres a fast-drying coating solution and a slow-drying coating solution, the two solutions containing the same binder and softeners dissolved in the same solvent.

14. The method of making a stencil sheet comprising successively applying to a porous base a solution of nitrocellulose in a relatively large amount of volatile solvent and a solution of nitrocellulose in a relatively small amount of volatile solvent, the first solution containing sufficient softening agent to produce a displaceable but relatively hard film, and the second solution containing sufficient softening agent to produce a soft and fluent film.

15. A stencil sheet comprising a porous fibrous base having a unitary displaceable coating consisting of a sizing layer and an external layer of different degrees of hardness, said layers being compatible and merging into one another.

16. The method of making a stencil sheet which comprises applying to an open base of porous fibres a quick-drying solution containing binder and softener, and, after said solution has partly dried in the base and before it has completely dried, applying a compatible slow-drying solution containing binder and softener.

NIELS HOLGER BJERG.  
ALBERT B. DICK, JR.